

April 19, 1932.

J. B. GRENALE

1,854,790

PROCESS AND MEANS FOR METAL DEPOSITING

Filed Jan. 24, 1930



Fig. 2.



James B. Grenale  
INVENTOR.

BY

William E. Varney  
ATTORNEY.

## UNITED STATES PATENT OFFICE

JAMES B. GRENALE, OF BALTIMORE, MARYLAND, ASSIGNOR OF ONE-HALF TO WILLIAM W. VARNEY, OF BALTIMORE, MARYLAND, AND ONE-HALF TO UNIVERSAL ALLOYS, INCORPORATED, OF BALTIMORE, MARYLAND, A CORPORATION OF MARYLAND

## PROCESS AND MEANS FOR METAL DEPOSITING

Application filed January 24, 1930. Serial No. 423,017.

The object of my invention is the depositing or plating of metals.

A further object of my invention is the depositing of alloys of metals on a metal of the same group of which one member of the alloy is a part.

A further object of my invention is an improved method of depositing metals.

A further object of my invention is an improved product of a deposited metal.

A further object of my invention is an apparatus provided with electrical means for carrying out my invention.

With the foregoing and other objects in view, my invention consists of the methods employed, combination and arrangements of systems, apparatus and means as hereinafter specifically provided, but it is understood that changes, variations and modifications 20 may be resorted to which come within the scope of the claims hereunto appended.

It is a recognized fact that plating articles in the ordinary bath does not produce a lasting coating when exposed to disintegrating 25 elements; for example, chrome plating on steel apparently gives very satisfactory results, but in time pitting or corrosion in spots occurs. Likewise, articles plated with nickel on iron show but short life when exposed to 30 weather conditions. I have discovered a new method of depositing metals on other metals in such action as will make the plating permanent.

I have discovered that using a plating metal, or an alloy of said plating metal alloyed with the metals to be plated disintegrated at the time of plating in a conveying bath and electrically deposited on the article to be plated, forms a kindred congenial association with kindred or like metals; at the same time, the metal being plated is not attacked by the conveying solution used, as the plated element is not a chemical component part of said solution unelectrically 45 energized.

To more fully understand my invention I will first describe the apparatus used in a small way and a number of the solutions used for different elements.

In the drawings of the herein described

apparatus embodying features of my invention, and which may be used in the practicing thereof and the production of the product involved, Figure 1 is a cross-section in elevation taken through 1-1 of Fig. 2, and 55 shows a preferred desired position of the respective parts involved; but these positions may be varied at will to a very large extent; Fig. 2 is a plan view of the apparatus shown in Fig. 1. The apparatus I am describing is 60 a lead lined tank of substantially 3 ft. square by about 2 ft. deep. These figures are given simply for illustrative work to convey an impression of the apparatus used.

Similar numerals refer to similar parts 65 throughout the several views.

1 is a wooden tank lined with lead 2. 3 is a stuffing box in the lower part of the tank for the introduction of an electrode; this stuffing box is insulated from the tank by 70 insulation 4. 5 is a supporting clamp resting upon support 6 and insulated therefrom by insulation 7. 8 is a rod or support resting upon the top of the tank or lead covering, but insulated therefrom by insulation 9 75 and is itself an electric conductor.

On rod or support 8 are hung the articles 10 to be plated, as shown, an automobile headlight. These are supported by conducting wires 11, or other suitable means; wires for 80 illustrative purposes are much simpler than clamps or rigid supports, which may be used, if desired, at the anode terminal. To these articles 10 a plus terminal 12 is attached of 85 a direct current electrical circuit, as shown in the drawings by means of connecting wires 11 and rod 8. 13 is the negative, or cathode, terminal of a direct current electric circuit of which 10 is the positive terminal, or anode. This terminal operates through stuffing box 90 3 and is insulated from tank 1 and lining 2. 14 are plates, bars or other forms of metal to be plated on deposited upon the anode 10. These plates are clamped on to carrier 15 by 95 any convenient means, as shown simply hung on the carrier; but it is preferable to have a better contact and that is attained by clamping the plates to lugs on the carrier.

Carrier 15 and its vertical posts 16 are electric conductors which are operated through 100

and supported by supporting clamp 5, and are clamped therein and regulated by clamping screw 17. To this vertical post 16 is attached the conductor to either side of a 110 bolt 5 3-wire alternating house circuit, the ground or neutral wire 19 of which is secured to the lead lining of the tank, grounding the same at 20; any alternating circuit, however, would function.

10 Having thus described an apparatus in which my process may be practiced, I will now describe a plating operation; as an illustration, I will take the article 10, made of iron or steel, as an automobile headlight to 15 be plated with chromium.

The plating metal 14 consists of chrome ferric alloy, preferably plates made of an alloy, of 70% chromium and 30% iron. The negative terminal, or cathode, 13 that I would 20 use in this case would be of iron. The tank is partially filled with a solution of the following: Precipitated 200 grammes of



25 plus 24H<sub>2</sub>O with NH<sub>3</sub>. Wash the hydroxide and dissolve in 120 grammes chromic acid dissolved in 2000 cu. cent. H<sub>2</sub>O. This bath should be preferably maintained at a temperature of 40° C. Current should be 30 used for about forty minutes in the alternating circuit coming from terminal 18, and a slow direct current of about 12 amperes flowing at the same time.

I have discovered that the direct terminals 35 should be as near the bottom of the tank as practicable; likewise, the articles to be plated, with a considerable depth of the solution above them.

I have discovered that plating on a metal 40 from a similar metal containing the major metal to be plated forms a very tough amalgamation, if I may use that expression, coating.

If it is desired to plate with nickel, plates 45 14 would be of a pure electrode nickel; if plating upon iron 10, an electrode 13 would also be of iron, and the following solution would be used in the tank:

50 NiSO<sub>4</sub> + 7H<sub>2</sub>O 75 grammes, MgSO<sub>4</sub> + 7H<sub>2</sub>O 15 grammes, H<sub>3</sub>BO<sub>3</sub> 15 grammes, H<sub>2</sub>O 1000 cu. cent. This bath should be maintained at 20° C., and the alternating current from terminal 18 should be run twenty minutes and 55 a direct current of 2 amperes for the same length of time.

If plating with cobalt is desired on iron, using an iron terminal 13, plates 14 should be made of cobalt, and the following solution 60 used in the tank:

CoSO<sub>4</sub> + H<sub>2</sub>O, 175 grammes, H<sub>2</sub>O 1000 cu. cent.; the bath should be maintained at a temperature of 15° C., using from two to four amperes direct current between terminals 13 65 and 10, and alternating current from ter-

70 minal 18, both currents simultaneously for about 30 minutes.

If it is desired to plate with cadmium on iron 10 with the iron terminal 13, the plates 14 are made of cadmium and the solution in the tank is as follows:

75 Cd(CO<sub>3</sub>)<sub>2</sub> 12 grammes, KCN 35 grammes, H<sub>2</sub>O 1000 cu. cent. This solution should be maintained at a temperature of 15° C. and a direct current of from 1 to 2 amperes should flow from the terminals 13 to the terminal 10 while an alternating current flows from terminal 18 for 30 minutes.

In the above, I have given four examples 80 of coating on iron with elements in a solution that will not attack the iron.

85 While I have used iron as illustrated, I do not wish to limit myself to the same, as any conducting metal, or any surface rendered conductive, may be plated upon with my apparatus and by my process. While I have shown the preferable solutions for the various alloys used, it is not necessary that the solution attack in any way the terminals 10 and 13; but, on the contrary, it is very desirable 90 that the solution should not attack these terminals. It is desirable that the solution should attack the plates or elements 14; this, however, is not absolutely essential, as the alternating current does the work at these terminals, and the direct current appears to be the conveying agent. The alternating current is controlled as desired by any well known means; I have shown a resister, 21.

95 As an illustration, I will plate on copper at terminal 10, using an iron electrode at 13 and chromium ferric as described in the first example given above for plates 14 and the solution above mentioned for chrome plating; the copper will be thoroughly plated, probably not as intimately associated with the plating as the iron would be. It will be preferable in this example to use a ferric chrome alloy, and also, preferably, a terminal 110 100 of copper.

105 While I have shown and described as a specific example an alternating circuit in which plate 14 is in circuit, a direct current may be used for disintegrating purposes through said plate 14; and while I have shown the lead lining 2 in said circuit, this terminal may be an independent removable terminal.

110 While I have shown terminal 13 as removable, I can use the tank lining 2 for this terminal.

I do not wish to be limited to any arrangement of the terminals, or to the character of current used.

115 Having thus described my invention, what I claim and desire to secure by Letters Patent is:

120 1. An electric plating means consisting of the metal to be plated operated upon by an alternating current of electricity in circuit with a disintegrating bath for said metal, an 125 130

object to be plated in said bath operated upon by a direct current of electricity the circuit of which comprises said bath, said object to be plated and means for contacting with said bath independent of the circuit of said alternating current whereby an element in said bath is deposited on said object.

2. An electric plating means consisting of the metal to be plated operated upon by an alternating current of electricity in circuit with a disintegrating bath for said metal, an object to be plated in said bath operated upon by a direct current of electricity the circuit of which comprises said bath, said object to be plated and means for contacting with said bath independent of the circuit of said alternating current whereby an element in said bath is deposited on said object, both of said currents operating at the same time but from different terminals respectively.

20 3. In a plating bath a plurality of electric circuits, one a disintegrating current to disintegrate the element to be deposited, another a depositing current for depositing the disintegrated element on an object to be plated but from different terminals respectively, both of said currents operating at the same time but from different terminals respectively.

25 4. The process of depositing an alloy on an object to be plated consisting of disintegrating the alloy in a disintegrating element thereof, by an alternating electric current one pole of which consists of the alloy to be disintegrated and the other pole of which comprises a contacting means in said disintegrating element, and then depositing the disintegrated alloy from said disintegrating element on to the object to be plated by electric means independent of the disintegrating means.

40 JAMES B. GRENALE.

45

50

55

60

65